

3,495,392

## BULKY DYED YARNS

Raymond J. Elia, Geneva, Switzerland, and George D. Null, Landenburg, Pa., assignors to E. I. du Pont de Nemours and Company, Wilmington, Del., a corporation of Delaware

No Drawing. Continuation-in-part of application Ser. No. 671,602, Sept. 29, 1967. This application June 26, 1968, Ser. No. 740,037

Int. Cl. D02g 3/02; D02j 1/22; C08g 19/00

U.S. Cl. 57—140

4 Claims

10

### ABSTRACT OF THE DISCLOSURE

Dyed synthetic polycarbonamide yarns are prepared that are suitable for the production of woven fabrics having the visual and tactile aesthetics of silk yarn-dyed fabrics.

### BACKGROUND OF THE INVENTION

This application is a continuation-in-part of application Ser. No. 671,602, filed Sept. 29, 1967.

Yarn-dyed natural silk fabrics are stiff and not excessively supple. Because of this relatively stiff nature, these fabrics are ideally suited for fabrication into women's gowns and dresses of outstanding quality. However, garments made of natural silk, although having outstanding appeal, lack the durability characteristics of garments made from synthetic filaments.

Numerous attempts have been made to prepare silk-like fabrics from synthetic polyamide yarns. Recently yarn has been developed which comprises a plurality of oriented synthetic continuous polyamide filaments at least some of which differ in shrinkability from other of said filaments. A particularly preferred yarn is the mixed filament yarn wherein both constituent types are polyamides derived from the PACM diamine family. Suitable PACM diamines include bis(4 - aminocyclohexyl)methane and bis 4 - amino(cyclohexyl)ethane. In yarn dyeing operations, mixed filament yarns from PACM polyamides tend to generate less shrinkage tension than other mixed continuous filament yarns. Consequently, the new PACM yarn as produced for use in piece-dyed fabrics are not entirely satisfactory for yarn dyeing on the commonly-used collapsible bobbins available in the textile trade. Dyed yarns prepared from mixed PACM yarns of this type when dyed on bobbins have very poor uniformity in bulk and dye-ability from the inside of the package to the outside. On the other hand, such yarns would be expected to be very useful if properly handled because of the development of differential shrinkage during the yarn dyeing operation.

### SUMMARY OF THE INVENTION

In accordance with the present invention a yarn is provided comprising a plurality of drawn, oriented synthetic polymer filaments, one group of which filaments differs in shrinkability from another group of said filaments, and all of which filaments consist of at least 50% by weight of polymer units of the formula



of the invention should exhibit a differential shrinkage between said groups of filaments of at least 1.5% when placed under a 4 milligram per denier load in boiling water for about 30 minutes, and said shrinkage differential should increase on heat setting at higher temperatures under the same load. The load is removed before making the DFL measurement as described below. The bulked yarn of the invention has a twist multiplier between 0.27 and 1.50, a liveliness multiplier less than 0.4, and has 3 to 10% differential filament length.

The yarn of the invention is prepared by twisting the specified mixed filament PACM polyamide yarn on conventional equipment to obtain a twist multiplier of about 0.27 to 1.5. The twist is then set by heating the yarn at constant length at a temperature of at least 70° C. but less than 105° C. to reduce the liveliness multiplier to below 0.4. Finally, the twist-set yarn is bulked by treating under shrinkage conditions at temperatures higher than in the twist-setting operation, thereby promoting the development of 3 to 10% differential filament length between the two filament species in the mixed filament yarn. Typical polymers for use in the yarn of the invention are the polyamides prepared from bis(4 - aminocyclohexyl)methane and sebacic, azelaic, or dodecanedioic acid.

The proportion of high to low shrinkage filaments required to obtain the desired results will vary depending on the difference in shrinkage potentials and on other factors such as filament denier, etc. In general, at least 25% by weight of the higher shrinkage filaments should be present and similarly at least 25% of the low shrinkage filaments should be present.

### DETAILS OF THE INVENTION

The different groups of filaments in the yarn which provide the prescribed differential shrinkage and resulting differential filament length in the yarn after shrinking, are provided by combining a first group of filaments consisting essentially of a polyamide having repeating units of Formula I and a second group of filaments consisting of a polyamide containing from 50 to 95 mol percent of the repeating units of Formula I and 5 to 50 mol percent of units of another polyamide prepared from a member of a class consisting of (1) the same diamine of Formula I with a different dicarboxylic acid and (2) the same dicarboxylic acid of Formula I with a different diamine. Physical differences between the two groups of filaments may also be used to promote differences in filament length.

The preparation of PACM polyamides is described in Gadecki and Speck U.S. Patent 3,249,591, Bolton & Kirk U.S. 2,512,606, and in British Patent No. 1,091,007. The mixed yarns preferably are spun by extruding the two polymer species from adjacent holes in the same spinneret. The mixed yarns are drawn and oriented by conventional methods.

In the process of the present invention the mixed filament PACM yarn is twisted on a conventional down-twister or up-twister to a twist multiplier level between about 0.27 and 1.50 allowing for shrinkage in the relaxed heat treatment later on. The twisted yarn is heat-treated (twist-set) on a bobbin or other rigid core at constant length to stabilize the yarn, i.e., to reduce liveliness in subsequent steps. Twist setting can also be done in a continuous process by running the yarn through a heated zone. The twist-setting may be done by exposure to wet or dry air at 70 to 105° C., but preferably by exposure to moist air. The temperature, moisture content, and time exposure are regulated to produce a yarn with a liveliness multiplier, as hereinafter defined, of less than 0.40, preferably less than 0.16.

In the next step the twist set yarns are treated at still higher temperature under very low tension to promote

wherein X is 1 or 2, Y is an integer in the range of 7-14 inclusive, R is the same or different and of the class of hydrogen and methyl, at least 40% by weight of the diamino polymer constituent being of a trans-trans stereoisomeric configuration. The yarn subjected to the process

65

70

development of differential filament length and increased bulk. Preferably the twist-set yarns are shrunk by heating under low tension with steam under superatmospheric pressure at a temperature of from about 120 to 140° C. The temperature should be sufficiently high to preclude any significant additional shrinkage during dyeing. Low tension may be assured by winding the twist set yarn in a uniform manner on a collapsible core and shrinking the yarn in package form in an autoclave.

The pre-shrunk yarn may then be dyed in a conventional manner. Preferably, it is package-dyed in an autoclave under superatmospheric pressure in the presence of a dye carrier for the filaments. Uniform dyeing is obtained by reversibly forcing the dye bath liquor through the package under pressure in a conventional manner. Through conventional techniques the twisted, dyed, bulked yarn may then be made into a fabric which requires no further stabilizing treatments such as heat-setting.

The woven fabrics of this invention upon removal from the loom are comprised of dyed yarns of filaments having a differential length of from about 3 to 10%. Yarns removed from the fabric have a substantially lower tendency to retain weave crimp, than do yarns removed from a piece-dyed fabric of similar construction. The fabrics of this invention have the stiffness and body of yarn-dyed fabrics prepared from natural silk combined with the performance and durability of synthetic polycarbonamide filaments. If desired, the fabrics may be softened by heat-setting at off-loom width at 170 to 190° C.

Yarn twist has a 2-fold role in this invention (1) to give the desired fabric aesthetics (e.g., higher twist-harder fabric, lower twist-soft fabric), and (2) to give good operability in packaging and weaving. For example, at least about 10 turns per inch (3.9 per cm.) are required in 60 denier warp yarns (twist multiplier 1.05) to get acceptable weaving, with at least about 2.5 turns per inch (0.99 per cm.) for 60 denier yarns in the fill (twist multiplier .27).

The yarns must not be so highly twisted that the twist restraining forces are so high as to prevent the desired differential filament shrinkage to occur. For this reason, a twist multiplier of 0.27 to 1.50 is normally preferred in the filling. Twist multiplier (T.M.) is defined as

$$T.M. = \frac{\text{Twist per inch} \times \sqrt{\text{yarn denier}}}{73}$$

$$T.M. = \frac{\text{Twist per cm.} \times \sqrt{\text{yarn denier}}}{(28.8)}$$

At twist setting temperatures or conditions other than those specified, yarn liveliness presents problems in handling, making uniform control difficult and creating undesirable non-uniformities in the resulting yarn and fabric. Higher twisting setting temperatures than those specified are detrimental to proper development of bulk and differential filament length during shrinking. Careful control of shrinking conditions is important. Sufficiently high temperatures must be employed to obtain the desired shrinkage differential between the filaments but conditions must not be so severe that undue degradation, discoloration, and loss of filament tensile properties results.

In a preferred embodiment of the process of this invention the treating steps are performed on the yarn package for convenience. The yarns are twisted and packaged and then subjected to the twist-setting operation in a conventional manner, for example in a heat-setting oven. The twist-setting facilitates yarn handling in package formation for the subsequent shrinkage treatment. The yarn must be shrunk under low tension for the proper amount of shrinkage to occur. Excessive variations in tension cause shrinkage variations and therefore variations in the differential filament length. In order to obtain sufficiently low shrinkage tension in package form the twist-set yarn may be wound on an easily compressible core, for example a collapsible paper core. The amount of shrinkage

which results is dependent on the yarn tension, temperature, pressure and time of exposure under the shrinkage conditions. The shrunk yarn is then substantially dimensionally stable throughout the following dyeing operation. This dimensional stability is necessary to insure uniform dyeing. Until the shrinkage step, the yarn handles like a normal straight, continuous filament yarn. During shrinkage the yarn shrinks and develops differential filament lengths. After shrinking the yarn is wound onto yarn-dye tubes and can be pressure dyed in a conventional manner, preferably with a suitable dye carrier such as butylbenzoate or lauryl alcohol. Dyeing under these conditions does not result in any substantial decrease in the differential filament lengths. The dyed yarns are wound onto cones with application of a lubricating oil to facilitate subsequent textile operations. The weaving or knitting is then performed in a conventional manner.

The packaging and winding operations in preparing these yarns can be done on any suitable winding equipment which gives uniform tension control and permits formation of relatively soft packages. Suitable equipment should give uniform tension control within the range of about  $\pm 0.5$  grams and permit formation of a package having a hardness in the range of 15-30 units as measured by a Type O-2 Durometer made by the Shore Instrument Company of New York.

To insure acceptable levels in uniformity of shrinkage in package form, packages should have hardness levels in the 15-20 range for 30 denier counts and 20-30 hardness levels for 60 denier yarn counts when measured in the form of a 0.4 lb. package. Yarn running tensions in the 0.5-1.0 range for the 30 denier counts and 1.5-3.0 grams for the 60 denier count are suitable.

The yarn packages are preferably shrunk by heating in an autoclave with superatmospheric steam at a temperature of 120 to 132° C., for example for 30 minutes. Such conditions sufficiently stabilize the yarn so that little additional shrinkage will occur during dyeing. A typical autoclave shrinkage cycle for 0.4 lb. packages is 35 three minutes under vacuum of 27 inches (75 mm.) of mercury, injection of steam at 127° C. for 30 minutes under a pressure of 26 lbs./in.<sup>2</sup> gauge (2.9 kg./cm.<sup>2</sup>) followed by vacuum as above for 8 minutes and release of vacuum over a period of 2 minutes. The resulting yarn packages show uniform shrinkage throughout. The actual shrinkage level obtained will be dependent upon the nature of the filaments in the yarn. Normally total shrinkage levels of 10-12% are suitable resulting in a differential filament length of about 7-8%. At lower levels of total shrinkage, correspondingly lower degrees of differential filament length will result.

The yarns used for this invention contain filaments which differ in length as the result of different shrinkages. The percent difference in filament length (DFL) between 55 the high and low shrinkage filaments is determined by cutting a 40 cm. strand from the yarn package after shrinking, doubling the strand, and tying the free ends together to form a loop about 19 cm. long. The free ends above the knot are taped to a vertical meter rule and the 60 lengths of isolated individual filament loops are measured by hanging a 0.4 milligram per denier weight in a loop. At least 5 low shrinkage and 5 high shrinkage filaments are measured in this manner. Percent DFL is calculated from the following equation:

$$\text{Percent FDL} = \frac{100(L_2 - L_1)}{L_1}$$

where  $L_2$  is the average length of the longer filaments and  $L_1$  is the average length of the shorter filaments.

For measurement of DFL on the shrunk twisted yarns a different procedure was used. A 20 inch length of yarn was doubled and the free ends tied and taped to a vertical meter rule. A 0.6 gram paper clip was employed as a weight to straighten the yarn. The yarn length ( $L_1$ ) was then measured. The yarn was then extended by pulling

on the paper clip until the point where all evidence of loopiness disappeared and the yarn length ( $L_2$ ) was measured. These values are then inserted into the percent DFL equation.

Twist liveliness of (T.L.) is determined at 21° C. and 75% relative humidity. Samples are removed tangentially from the package by rolling the package so that no twist is added or removed. A pointed weight of 1 g. is fastened to one end of a suspended strand which is of known length (about 10 cm.). The yarn is allowed to untwist as a result of the action of the weight. The number of turns is counted during unwinding to an equilibrium point. Any rotation past the equilibrium point is not counted by taking the net number of turns to equilibrium. The twist liveliness is finally calculated by dividing the net turns to equilibrium by the original length of the test sample in cm. before unwinding. The answer is expressed in turns/cm. In 60 denier yarns of the invention, the twist liveliness is below 0.6 turns/cm.

All yarns of the invention have a liveliness multiplier below 0.4, preferably below 0.16. The liveliness multiplier (L.M.) is a factor which relates twist liveliness to denier:

$$L.M. = \frac{T.L. \times \sqrt{\text{denier}}}{28.8}$$

Yarns of equal liveliness multiplier have approximately an equal ability to kink during the relaxed heat treatment (e.g., on collapsible bobbin). Liveliness may be also judged subjectively as in Example I.

The following examples illustrate the present invention.

#### EXAMPLE I

As a starting material there was prepared by co-spinning through separate holes in a single spinneret a mixed shrinkage yarn of about 60 denier and containing 36 filaments. Eighteen of the filaments were a polymer of bis(4-aminocyclohexyl)methane containing 70% by weight of trans-trans-isomer and dodecane dioic acid, and the other eighteen filaments were a copolymer of the same diamine with 90 weight percent dodecane dioic acid and 10 weight percent of isophthalic acid. The fila-

show uniform development of DFL throughout the package.

The twist-set shrunk yarns were wound without difficulty into dye packages at 0.5 gm. tension onto perforated stainless steel tubes for pressure dyeing. The yarns were 5 scoured and then pressure dyed in a conventional package dyeing manner, dyeing at 240° F. (115.5° C.) for 90 minutes with 5% "Resolin" Blue FBLD (Color Index Disperse Blue-71) and 5% (on weight of fiber) "Charlab" DAC-888, a commercial butyl benzoate dye carrier. 10 There is substantially no change in yarn DFL upon dyeing. No dye non-uniformity (dye junction) is observed in satin fabrics in which outside, middle and inside yarns from the dye package are woven side-by-side.

15

TABLE I

|                                  | A    | B   | C   | D   | E    | F   |
|----------------------------------|------|-----|-----|-----|------|-----|
| Twist-set temp., °C.:            |      |     |     |     |      |     |
| Dry bulb.....                    | 71   | 77  | 82  | 88  | 93.5 | 104 |
| Wet bulb.....                    | 64.5 | 70  | 76  | 80  | 86   | (*) |
| Subjective twist liveliness..... | 5    | 3   | 2   | 2   | 1    | 0   |
| Yarn DFL (percent):              |      |     |     |     |      |     |
| After preshrinkage.....          | 8.5  | 6.8 | 5.2 | 5.0 | 4.8  | 3.6 |
| After dyeing.....                | 7.5  | 6.5 | 6.5 | 5.3 | 4.9  | 3.7 |

\*Saturated steam.

#### EXAMPLE II

25 An 8-hardness satin fabric was woven using the dyed yarn prepared as described in Example I B for the filling. The yarn had been twisted 5 turns/inch Z. (1.97 turns/cm.) and set as described at 77° C. and pre-shrunk at 126° C. The yarn had a DFL of 6.5%. Two ends of this 30 yarn were plied and twisted 2.5 S turns/inch (0.785 turns/cm.) in the ply. The warp yarn was prepared as in Example I, but with 30 denier 18 filament with 15 turns Z twist per inch (5.9/cm.). The warp was twist set and shrunk under the same conditions as the filling. The fabric was of 3.74 oz./yd.<sup>2</sup> (126.7 gms./meter<sup>2</sup>) construction having 350 ends/inch warp and 98 picks per inch fill (138 ends per cm. warp and 40 picks per cm. fill).

35 Fabric properties off the loom, after framing at off-loom width at 149° C. for 1 minute, after heat-setting at off-loom width at 180° C. for 30 seconds followed by 1 minute at 190° C. and after semi-decating 1 minute with steam—2 minutes vacuum, are shown in Table II.

TABLE II

| Fabric property                                              | Off loom     | Framed     | Heat-set     | Semi-decated after heat-set |
|--------------------------------------------------------------|--------------|------------|--------------|-----------------------------|
| Weight, oz./yd. <sup>2</sup> (gms./meter <sup>2</sup> )..... | 3.74 (126.7) | 3.55 (120) | 3.47 (126.7) | 3.47 (126.7)                |
| Bending length (cm.):                                        |              |            |              |                             |
| Warp.....                                                    | 1.9          | 1.85       | 1.62         | 1.56                        |
| Fill.....                                                    | 1.75         | 1.72       | 2.43         | 2.18                        |
| Flexural rigidity (mg.-cm.):                                 |              |            |              |                             |
| Warp.....                                                    | 88.8         | 77.1       | 50.0         | 45.3                        |
| Fill.....                                                    | 68.0         | 62.1       | 169.6        | 121.9                       |

55 The unexpected extent and kind of fabric response to heat-setting, with the warp and fill responding in opposing directions, is readily apparent from the data. As shown by the flexural rigidity, fabric firmness of hand increases markedly in the fill and decreases in the warp upon heat-setting above 350° F. (180° C.).

60 Bending length is defined as the length, in cm. of a strip of fabric of unit width which would be required as a horizontal cantilever to cause the fabric to leave its support on a curve having a unit radius.

65 Flexural rigidity, derived from the bending length and the weight per unit area of the fabric, is defined as the moment of couple required to bend a strip of fabric of unit width in a circle having a unit radius. It is calculated from the product of the bending length and weight per unit area of the fabric. This value increases as the firmness of hand of the fabric increases.

70 The fabric samples are cut so as to measure these values in both the warp and fill directions. Bending length is measured by means of a strip of fabric suspended in a heart-shaped loop (a double cantilever). The heart loop test is described in ASTM Standards 1958, Part 10, published by the American Society for Testing Materials,

75

ments were of a symmetrical trilobal cross-section and contained 2% of a finely divided kaolinite. This yarn was a mixed shrinkage yarn because the copolymer filaments have higher shrinkage than the homopolymer filaments when co-spun and drawn under the same conditions. Uptwist packages containing 0.4 lb. of this yarn having 5Z twists per inch were twist set for 90 minutes under the conditions shown in Table I. Yarns from the twist-set packages were subjectively rated for yarn twist liveliness on a scale where 5 is lively and 0 is substantially dead or no twist liveliness with the results shown in Table I. The yarns were then uniformly wound on collapsible paper cores into packages (for shrinking) at 0.5 gm. tension to give a package hardness of 20 units.

The yarn packages are then shrunk in an autoclave with steam at 127° C. for 30 minutes. A non-twist-set control yarn develops 8-9% differential filament length (DFL) due to the mixed shrinkage. The yarn twist-set at 160° F. (71° C.) (dry bulb temperature) shows about the same DFL; higher twist-set temperatures result in reduced DFL; however, the DFL remains acceptable for a twist-set temperature up to 220° F. (104° C.) as shown in Table I. The packages from yarn twist-set at 71-104° C.

Philadelphia, Pa., pages 557-562. It has the ASTM test designation: D1388-55T, Method B. A fabric sample 1 x 6½ inches (2.54 x 16.5 cm.) is used, cut to measure properties for the warp and fill directions as prescribed. The sample is mounted such that the measured specimen length is 6 inches (15.24 cm.).

What is claimed is:

1. Process of preparing a continuous filament yarn by twisting a yarn comprising filaments having differential shrinkages, setting the twist while maintaining the yarn at substantially constant length and thereafter heating the yarn under conditions permitting shrinkage of the yarn characterized in that

(a) the yarn comprises a plurality of drawn, oriented synthetic polymer filaments, at least some of which filaments differing in shrinkability from others of said filaments, all of which filaments consist of at least 50% by weight of polymer units of the formula



wherein X is 1 or 2, Y is an integer in the range of 7-14 inclusive, R is the same or different and of the class of hydrogen and methyl, at least 40% by weight of the diamino polymer constituent being of a trans-trans stereoisomeric configuration, said yarn when subjected to boiling water exhibiting a differential shrinkage between said filaments of at least 1.5% under a load of 4 milligrams per denier said shrinkage differential further increasing upon subsequently subjecting said yarns to higher heat-setting temperatures in the dry state under the same load,

(b) the setting of the twist is carried on at a temperature in the range from 70-105° C.,

(c) the shrinkage step is carried on at a higher temperature than the temperature of the twist setting and under conditions of temperature and tension

such that from 3-10% differential shrinkage between at least two groups of filaments develops and such that substantially no further shrinkage takes place during any subsequent dyeing.

2. The process of claim 1 wherein the differentially shrunk yarn is dyed prior to producing fabric therefrom, said shrinkage step conditions being such that substantially no further shrinkage takes place during dyeing.

3. A yarn of at least two groups of filaments, the filaments in one of said two groups differing from 3 to 10% in length from the filaments of the other of said two groups, the filaments in both said groups consisting of at least 50% by weight of polymer units of the formula:



wherein X is 1 or 2, Y is an integer in the range of 7-14 inclusive, R is the same or different and of the class of hydrogen and methyl, at least 40% by weight of the diamino polymer constituent being of a trans-trans stereoisomeric configuration, the said yarn having a twist multiplier between 0.27 and 1.50 and a liveliness multiplier of less than 0.4.

4. The yarn of claim 3 wherein said two groups of filaments each comprise at least 25% of the filaments in the yarn.

#### References Cited

##### UNITED STATES PATENTS

|           |         |        |       |        |
|-----------|---------|--------|-------|--------|
| 3,225,534 | 12/1965 | Knospe | ----- | 57-140 |
| 3,416,302 | 12/1968 | Knospe | ----- | 57-140 |
| 3,438,192 | 4/1969  | Ryan   | ----- | 57-140 |

JOHN PETRAKES, Primary Examiner

U.S. Cl. X.R.

57-157; 28-72.17; 260-78